

Feb. 10, 1959

H. C. BRASSFIELD ET AL

2,872,719

METHOD OF FABRICATING SMALL SPHERICAL PELLETS

Filed Sept. 25, 1957



INVENTORS  
HENRY C. BRASSFIELD  
CARL T. DURHAM JR.  
BY

*Roland A. Goodman*

ATTORNEY—

1

2,872,719

## METHOD OF FABRICATING SMALL SPHERICAL PELLETS

Henry Clay Brassfield, Fosters, Ohio, and Carl T. Durham, Jr., Roanoke, Va., assignors to the United States of America as represented by the United States Atomic Energy Commission

Application September 25, 1957, Serial No. 686,268

13 Claims. (Cl. 25—156)

This invention deals with a method and apparatus for the fabrication of small spherical shot type pellets, and in particular with a method and apparatus for the formation of spherical pellets from ceramic or refractory materials.

In the prior art, spherical pellet formation is affected by several methods, chiefly by dropping from shot towers, by the use of centrifugal force, or by molding. One great disadvantage inherent in all of these above mentioned methods for spherical pellet formation is the fact that it is extremely difficult to control the size of the pellets with any great degree of exactitude. Another disadvantage is that none of these methods is particularly adapted to the production of very small spherical pellets. The present invention accomplishes spherical pellet formation by a new and radically different method, which method is particularly applicable to the formation of extremely small spherical pellets.

An object of this invention is to provide a method and apparatus particularly adapted to effect the production of large quantities of small spherical pellets conveniently and economically.

A further object of this invention is to provide a method and apparatus particularly adapted to effect the production of small spherical pellets, wherein the range of pellet sizes may be easily and automatically controlled thus insuring a consistently uniform product.

These objects are accomplished by preparing a suspension, or slip, of powdered ceramic material and water with a controlled pH, dropping the suspension through a small capillary into a moving bed of water-repellent powder, drying the spherical drop on the moving bed, separating the spheres from the bed powder, and firing the spheres at 1500° C.—1800° C. to form a dense body.

For a more full and complete understanding of the subject invention, reference is now made to the drawing of an apparatus designed for the practice of this invention.

In Figure 1; the capillary tube, at the tip of which the drops of ceramic suspension form, is designated as 1, a container for the slip or suspension which is positioned above and connected to the capillary tube is designated by 2 and 3 designates a conveyor belt which carries the moving bed of water repellent powder 4. The powder hopper 5 and stationary guides 6, provide for the deposition of this moving bed of water repellent powder on the upper surface of the belt. A battery of infra red lamps 7, is positioned over the belt and a screening element, 8, is located at the end of the conveyor belt, wherein the spherical pellets are separated from the water repellent powder. A voltage supply is designated by 9 and the cable connecting the voltage supply to the slip container as 10.

In operation the water repellent powder is loaded into hopper 5, from which it falls in a thin stream onto the moving belt 3 which is positioned below the hopper. This powder is shaped into a narrow strip by the stationary guides 6. The narrow bed of water repellent powder is then carried underneath the capillary tip 1, by the mo-

2

tion of the conveyor belt 3, and as drops of ceramic containing slip form on the tip of the capillary tube 1, they are deposited on the surface of water repellent powder 4.

5 The water repellent properties of the powder cause these small drops to assume spherical shape, and while retaining this spherical shape, the pellets are carried under the battery of infra red drying lamps 7. Here the water is evaporated away from the pellets. The slightly damp ceramic spheres are then carried to the separatory screen 8. Here 10 the water repellent powder falls through the screen while the pellets are retained upon it. The spherical pellets are then collected and fired to produce the finished product.

The capillary-drop apparatus consists of a plastic container, supported above the traveling powder bed, and 15 equipped with a small motor stirrer to maintain uniform dispersion of the suspension of water and ceramic material. The aluminum paddle of the stirrer is electrically insulated from the motor shaft by a plastic coupling, and the shaft is sealed at the container lid by means of a rubber gasket.

20 The size of the drop produced is controlled in three ways. The size is determined principally by the effective diameter of the capillary tip; however, this dimension having been fixed, variation may be secured by regulation 25 of gas pressure above the liquid and by application of an electrical charge to the slip.

The surface of the capillary tip upon which the drop forms should be kept as small as possible. This is accomplished by grinding the tip to a narrow lip. In addition, if the slip is permitted to wet the tip and stem of the capillary, it will creep up the outside wall of the tube and drops will form on a larger surface. Wetting may be prevented by the application of a water-repellent material. No detailed study of the relation of the capillary diameter to drop size has been made, but practice has shown that internal diameters from 0.012 to 0.018-inch yield drops within the desired size range.

Gas pressure is applied to the slip container primarily to control the dropping rate, but this in turn affects the 40 drop size. The gas is argon, which is first saturated with water to minimize evaporation of water in the slip and is then led through a pressure regulator to the apparatus. Pressure adjustment is manual, and the normal operating pressure of 0.5 to 2.0 p. s. i. is read on a 0-5 p. s. i. gauge.

45 More precise control of drop size is obtained by imposition of a high voltage between the slip and the water repellent powder bed. The voltage is applied to the slip, which is insulated from the ground, by means of a coaxial cable. The resulting effect upon droplet size demonstrates that adjustment over a fairly wide range is possible. While we do not wish to be restricted by theory, the phenomenon of drop size control by the D. C. voltage probably results from a combination of the Coulomb forces between the positively charged drop and the negative bed, 50 and a reduction of the surface tension of the forming drops by the accumulation of positive charges on its surface. To form the drops, potentials between 500 and 4000 volts have sufficed.

55 Many ceramic materials are suitable for treatment by this process, specifically alumina ( $Al_2O_3$ ), beryllia ( $BeO$ ), uranium dioxide ( $UO_2$ ), and molybdenum disilicide ( $MoSi_2$ ), or mixtures of these materials or other ceramic materials. However, the ceramic material actually used must be in a very finely divided state. For example the dried  $MoSi_2$  pellets produced by this method will not sinter to a satisfactorily dense body on firing unless the  $MoSi_2$  has been ground to an average particle size of 13.0 microns or less.

60 The creation of a well-formed sphere by the capillary-drop method depends upon the properties of the slip or

suspension, of which the most important is its degree of deflocculation, as controlled by its pH. If the slip is deflocculated, a dimpled sphere results on drying. In practice, a pH between 1.6 and 2.2 is preferred and is obtained by adding the necessary quantity of concentrated hydrochloric acid to the slip just before it is placed in its container.

To obtain good dropping characteristics from the capillary, the slip should also be of the correct viscosity. With a typical 0.014-inch-diameter capillary, a slip having a viscosity between 1,500 and 2,400 centipoises is preferred. Any lower value tends to produce a continuous stream from the capillary, and a higher viscosity produces low rates of dropping.

The pH of the slip and its viscosity are mutually dependent properties, but some degree of freedom may be obtained by a variation of a third important slip property, specific gravity. By the correct selection of liquid-to-solid ratio the desired viscosity may be obtained within the required pH range. The specific gravity of the slip is also independently important; if it is too low, drying of the drops will not take place in a convenient length of time.

There are several readily available powders which will resist wetting by water. Some powders which were tested are; stearated aluminum metal powder, micro-pulverized graphite, carbon black, and lycopodium powder. Stearated aluminum powder was selected because of its low cost, cleanliness, and ease of removal from the pellets via evaporation or oxidation during firing in a wet hydrogen atmosphere.

The feeding of the powdered aluminum onto the moving conveyor belt in the form of a bed of uniform powder density presented some difficulty. During simple gravity feeding, the aluminum powder displayed an erratic tendency to bridge over the feed orifice and it became necessary to install a vibratory feeder. This device drops a continuous stream of powder onto the belt, the rate of feeding being controlled by varying the amplitude of vibration. Once on the belt, the powder is shaped into the desired form by stationary guides. The precise scheduling of the feed rate relative to the conveyor belt speed requires periodic attention and adjustment of the feed.

The conveyor system comprises a 2-inch, 3-ply rubber canvas belt resting in an aluminum channel beam and driven by a variable speed transmission, capable of producing belt speeds from zero to 42 feet per minute. The normal belt speed for the operation is from three to four feet per minute. After passing the capillary dropping station, the belt carries the spherical drops under four infrared heating units, where they are dried. To avoid overheating the rubber belt, the bottom half of the channel beam in which it rides was closed and watercooled.

The drying system consists of four infrared heating units arranged over the far end of the conveyor belt. Control of the drying rate may be obtained by varying the height of the heaters above the bed and by controlling the voltage input to the heaters. Drying is regulated to produce damp-dry spherical pellets, because pellets which are completely dried have a tendency to break as they are screened.

A screening system is placed at the discharge end of the conveyor belt to separate the dried pellets from the aluminum powder. The 14 x 20 mesh screen is vibrated at fixed intervals by an automatic control system, and care is taken to leave a cushion of aluminum powder on the screen to prevent breakage of the pellets when they fall onto the screen from the belt. The fine particle size of the water repellent powder makes it mandatory to enclose the screening apparatus and to exhaust the chamber by means of a fan. The water repellent powder is reclaimed and fed back into the powder feed mechanism. The belt is cleaned by rotating brushes incorporated into the screening unit.

The dried pellets are placed in a suitable crucible and fired in a hydrogen atmosphere furnace. Firing tempera-

tures are dependent on the material used for the pellet; however, firing temperatures in the range of 1500° C. to 1800° C., holding at temperature for one to two hours, are generally sufficient to properly mature the pellets.

5 The invention is illustrated, but is not intended to be limited, by the following examples:

#### Example I

The slip used was composed of acid-leached alumina 10 and water. The slip was used at pH of 1.6 and a specific gravity of 2.42, and was dropped at a rate of approximately 240 drops a minute. The fired diameter of these alumina spheres was approximately 0.067 inch.

#### Example II

A water suspension of very fine molybdenum disilicide was prepared by adding molybdenum disilicide to water until the specific gravity of the resultant slurry was 3.37 gms./cc. Concentrated hydrochloric acid was added until the pH of the slurry was 2.1. Using 2 p. s. i. argon pressure, 0.100 inch diameter spheres of molybdenum disilicide were formed at a rate of from 60 to 80 per minute.

25 Although the present invention has been described with reference to the specific details of certain embodiments thereof, it is not intended that such details shall be regarded as limitations upon the scope of the invention except insofar as included in the accompanying claims.

We claim:

- 30 1. A process for producing spherical pellets of material, which consists of powdering the material to be pelletized, forming a suspension of this powdered material in a liquid carrier or vehicle, causing small drops of this suspension to rest upon a surface of liquid repellent powder, drying the drops of suspension, and collecting and firing the spherical pellets thus formed.
- 35 2. A process according to claim 1 wherein the liquid carrier or vehicle is water.
- 40 3. A process for producing spherical pellets of material, which consists of powdering the material to be pelletized, forming a suspension of this powdered material in a liquid carrier or vehicle, forming small drops of this suspension at the tip of a capillary tube, causing these drops to rest upon a surface of liquid repellent powder, drying the drops of suspension, and collecting and firing the spherical pellets thus formed.
- 45 4. A process according to claim 3 wherein the liquid carrier or vehicle is water.
- 50 5. A process for producing spherical pellets of ceramic material, which consists of powdering the ceramic material to be pelletized, forming a suspension of this powdered ceramic material in a liquid carrier or vehicle, causing small drops of this suspension to rest upon a surface of liquid repellent powder, drying the drops of suspension, and collecting and firing the spherical pellets thus formed.
- 55 6. A process according to claim 5 wherein the liquid carrier or vehicle is water.
- 60 7. A process for producing spherical pellets of ceramic material, which consists of powdering the ceramic material to be pelletized, forming a suspension of this powdered ceramic material in a liquid carrier or vehicle, forming small drops of this suspension at the tip of a capillary tube; causing these drops to rest upon a surface of liquid repellent powder, drying the drops of suspension, and collecting and firing the spherical pellets thus formed.
- 65 8. A process according to claim 7 wherein the liquid carrier or vehicle is water.
- 70 9. A process according to claim 5 wherein the powdered ceramic material comprises finely divided aluminum oxide ( $Al_2O_3$ ).
- 75 10. A process according to claim 5 wherein the powdered ceramic material comprises finely divided beryllia ( $BeO$ ).

11. A process according to claim 5 wherein the powdered ceramic material comprises finely divided uranium dioxide ( $UO_2$ ).

12. A process according to claim 5 wherein the powdered ceramic material comprises finely divided molybdenum disilicide ( $MoSi_2$ ).

13. A process according to claim 5 wherein the powdered ceramic material is any mixture of aluminum oxide, beryllia, uranium dioxide, or molybdenum disilicide.

## References Cited in the file of this patent

## UNITED STATES PATENTS

|           |                  |               |
|-----------|------------------|---------------|
| 1,561,971 | Coffin et al.    | Nov. 17, 1925 |
| 1,773,257 | Buse             | Aug. 19, 1930 |
| 2,180,757 | Hermann          | Nov. 21, 1939 |
| 2,436,771 | Hood             | Feb. 24, 1948 |
| 2,562,149 | Mollring         | July 24, 1951 |
| 2,790,201 | Eilbracht et al. | Apr. 30, 1957 |
| 2,799,074 | Garloni          | July 16, 1957 |